

## UNITED STATES PATENT OFFICE.

RUDOLF AUERBACH, OF PROBSTDEUBEN, NEAR LEIPZIG, GERMANY, ASSIGNOR TO CHROMEPLATE, INC., OF UNION CITY, NEW JERSEY, A CORPORATION OF NEW JERSEY.

## ELECTROLYTIC DISPOSITION OF CHROMIUM.

No Drawing.

Application filed January 6, 1927. Serial No. 159,507.

My invention refers to the electrolytic deposition of metallic chromium, and its particular object is to provide means whereby such deposition can be carried through under 5 more favorable conditions and in a less expensive manner than was hitherto possible.

As is well known to those skilled in the art, an electrolytically produced deposit of chromium will be the denser and the more 10 homogeneous the lower the density of current employed in producing same. If the current density is too high, exceeding 5 ampères per square decimetre, the electrolytic deposit of chromium will be porous and brittle, so 15 as to readily splinter off the base material. Furthermore with such high current densities the separation of the metal will not occur in perfect purity, oxygen compounds being deposited in the pores which impair the qualities of the deposit. 20

On the other hand the yield of chromium per ampère hour is dependent from the current density, this yield increasing as the density of current increases. In order, therefore, 25 to obtain as strong a deposit as possible in the least possible time, the largest possible density of current is preferable.

I have now ascertained that if a solvated colloid is added to the solution of chromic acid 30 or chromates employed in the electrolytic process, a homogeneous deposition of chromium will occur over a far wider range of current densities. In other words, chromium will be deposited from the solution on the one 35 hand with so low densities of current, that under ordinary conditions no separation of metal would occur. On the other hand the range within which dense and firmly adhering deposits are obtained extends up to high 40 current densities (beyond 15 ampères per square decimetre), so that the high yield obtainable under these conditions, which amounts substantially to 30 per cent, can be utilized in a commercial manner.

In view, however, of the fact that most of the chromium solutions nowadays in use contain either chromic acid or chromates, it is impossible to employ organic colloids. For 45 while such colloids will at first act in the manner above described, nevertheless in consequence of the oxidation of the organic sub-

stances the composition of the solution will vary from time to time in such manner as to require constant watching and correcting.

I have now found that colloidal silicic acid 55 and colloidal silicates are particularly useful and effective in the direction aforementioned.

In carrying out my invention I may, for instance, proceed as follows:

## Example 1.

5 grams of soluble water glass ( $Na_2Si_4O_9$ ) of 28° Bé. are dissolved in 500 ccms. water, and to this solution is added under constant stirring a solution of 10 grams chromic acid 65 in 500 ccms. water. Only after the two solutions have been mixed in the manner aforesaid, the electrolytic solution is completed by slowly adding further quantities of chromic acid or chromates and the like. 70

## Example 2.

To a solution of 5 grams of soluble water glass ( $Na_2Si_4O_9$ ) in 500 ccms. water are added under stirring 500 ccms. of a dilute solution of a chromium salt, to which has been added sulphuric acid or some other suitable acid. In this manner is obtained a colloidal, highly viscous mixture of chromium silicate and silicic acid. Also in this case I prefer 80 dissolving the rest of the chromium salts only after the colloidal mixture has been finished.

If strong mineral acids have been used in the production of the silicates, it is preferable to subject the solutions to dialysis before preparing them ready for use, in order to free them from the dispersed particles which might cause trouble during the electrolytic process. 90

I wish it to be understood that I do not desire to be limited to the exact substances and operations above described for obvious modifications will occur to a person skilled in the art. 95

I claim:

1. The method of electrolytically depositing metallic chromium, which consists in adding to a solution containing chromic acid, soluble freshly made silicic acid and electrolyzing the solution. 100
2. The method of electrolytically deposit-

ing metallic chromium, which consists in adding about a 1% solution of soluble water glass ( $Na_2Si_4O_9$ ) to about a 2% solution of chromic acid, mixing the resultant solution with further quantities of a chromic acid and electrolyzing the solution.

3. The method of electrolytically deposit-

ing metallic chromium, which consists in adding soluble water glass ( $Na_2Si_4O_9$ ) in about a 1% solution to a dilute solution of a chromium salt to which has been added an acid and electrolyzing the solution.

In testimony whereof I affix my signature.

RUDOLF AUERBACH.